# EUROPEAN PATENT SPECIFICATION

(11) **EP 1 269 876 B1**
(45) Date of publication and mention of the grant of the patent: **09.12.2009**
(21) Application number: 02254526.3
(22) Date of filing: 27.06.2002
(51) Int. Cl.: A44B 19/00, A44B 18/00, A44B 17/00

(54) **Fastener product made of hydrolysis-resistent synthetic resin**
Hydrolysebeständiges Harz für Verschlussvorrichtung
Produit d'attachage en résine synthétique résistante à l'hydrolyse

(30) Priority: 27.06.2001 JP 2001194563
(43) Date of publication of application: 02.01.2003
(73) Proprietor: YKK Corporation, Chiyoda-ku, Tokyo (JP)
(72) Inventor: Kumano, Isamu, Kurobe-shi, Toyama-ken (JP); Hirota, Mutsuo, Shimoniikawa-gun, Toyama-ken (JP); Inamura, Toshiaki, Shimoniikawa-gun, Toyama-ken (JP); Aoshima, Hiromi, Kurobe-shi, Toyama-ken (JP)
(74) Representative: Luckhurst, Anthony Henry William

(56) References cited:
- EP-A- 1 229 061
- GB-A- 1 471 950
- US-A- 5 436 051
- US-B1- 6 230 373
- PATENT ABSTRACTS OF JAPAN vol. 015, no. 064 (C-0806), 15 February 1991 (1991-02-15) & JP 02 292318 A (KURARAY CO LTD), 3 December 1990 (1990-12-03)

## Description

### BACKGROUND OF THE INVENTION

### 1. Field of the Invention:

This invention relates to a fastener product made of a synthetic resin, which product is excellent in resistance to moist heat and resistance to hydrolysis. More particularly, the present invention relates to recyclable fastener products of synthetic resin such as slide fasteners of synthetic resin, which products are excellent in durability against wet heat and capable of maintaining the stable state of engagement without producing deterioration of strength even when repeatedly left under a high-temperature and high-humidity atmosphere.

### 2. Description of the Prior Art:

Most of the clothes such as working clothes heretofore used in a clean room of a pharmaceutical factory and those used in a hospital, medical service sites, nursing facilities, and the like are disposable. Since these clothes are disposed of by incineration as industrial waste after use, the desirability of reusing the clothes has come to find enthusiastic recognition year after year from the viewpoints of environmental pollution and saving of resources.

In order to reuse these products in the above-mentioned working places, the clothes must be washed and subjected to autoclaving (120-130°C x 30 minutes) with high-temperature and high-pressure steam as a sterilization treatment every day. Therefore, the products using the conventional polyester long fibers easily suffered hydrolysis by repeated processing and resulted in deterioration of strength.

In recent years, polyester fibers excelling in resistance to hydrolysis have been developed. As a result, the durability of the textile of a woven and/or knitted product against wet heat has been improved considerably, and under the present situation it is possible to provide the clothes which can be reused under the above conditions.

However, the above problems will also hold for the fastener products to be attached to the clothes. For example, a slide fastener made of a synthetic resin will be deteriorated by about 50 rounds of autoclaving due to hydrolysis and thus cannot be used any longer. Specifically, in the case of coupling elements of polyester, for example, the deterioration thereof due to hydrolysis with high-temperature steam proceeds during repeated use thereof for a relatively short period and autoclaving. Consequently, cracks, flaws, the fracturing phenomena into the shape of fiber and the like may occur in the engagement portions (heads) of the coupling elements, thereby causing deterioration of strength thereof. Eventually, the state of engagement of coupling elements will come off and the product will no longer function as a fastener. On the other hand, in the case of coupling elements made of nylon, although they have an advantage of hardly causing deterioration of the strength, they poses the problem of suffering discoloration in brown with the high temperature steam. Many of such a clothes include slide fasteners, see for example document US 6 230 373 B.

### SUMMARY OF THE INVENTION

It is therefore a fundamental object of the present invention is to provide a a slide fastener of synthetic resin, which product exhibits excellent durability against wet heat and is capable of maintaining the stable state of engagement without producing deterioration of strength, discoloration, etc. even when repeatedly left under the high-temperature and high-humidity atmosphere.

A further object of the present invention is to provide a recyclable slide fastener of synthetic resin, which product is excellent in both the resistance to moist heat and resistance to hydrolysis.

To accomplish the objects mentioned above, the fundamental mode of the present invention provides an engagement member made of a synthetic resin comprising an attachment part and an engagement part, which member is characterized by the fact that at least the engagement part mentioned above is made of a hydrolysis-resistant synthetic resin. The term "attachment part" as used herein refers to a part to which an engagement part is attached or a part to be utilized for attachment to the other products, such as a fastener tape of a slide fastener. And the term "engagement part" as used herein refers to such parts as coupling elements of a slide fastener.

Preferably, the hydrolysis-resistant synthetic resin material mentioned above is polyester having a carbodiimide-based hydrolytic stabilizing agent incorporated therein.

In accordance with a first embodiment of the present invention, there is provided a slide fastener made of a synthetic resin having a pair of fastener tapes and coupling elements fixed to the edges of the fastener tapes wherein the fastener tapes and the coupling elements are made of a synthetic resin material containing a bis-carbodiimide as a hydrolytic stabilising agent and said coupling elements are continuous coupling elements in a coiled or zigzag form.

When the slide fastener comprises sewing threads for the fixation of the coupling elements to the fastener tapes and/or core cords extended as inserted through the individual coupling elements in the longitudinal direction thereof, the sewing threads and/or the core cords may be made of a containing a bis-carbodiimide as a hydrolytic stabilising agent synthetic resin material.

Further, in the slide fastener of the type having upper and lower stop members provided respectively at the upper and lower ends of the rows of coupling elements, the upper and lower stop members may be made of a synthetic resin material containing a bis-carbodiimide as a hydrolytic stabilising agent as in the case of the other component parts mentioned above.

In the open-link type slide fastener which has a pin-and-box separator and a pair of reinforcing sheet-like members which have fixed to the lower end portions of the fastener tapes but having no lower stop member, the pin-and-box separator and the reinforcing sheet-like members mentioned above may be made of a synthetic resin material containing a bis-carbodiimide as a hydrolytic stabilising agent as in the case of the other component parts mentioned above.

In a preferred embodiment, in any of the cases mentioned above a slide fastener has substantially all the component parts thereof made of the same chemical type or system of material. Incidentally, the slider itself may be manufactured from a metallic material etc. and it has no problem in terms of resistance to hydrolysis. When the recycling use is taken into consideration, however, the slider may be made of the same chemical type of synthetic resin material as the other component parts mentioned above.

Since the fastener products of synthetic resin of the present invention, such as a slide fastener of synthetic resin are made of a hydrolysis-resistant synthetic resin, particularly polyester having a carbodiimide-based hydrolytic stabilizing agent incorporated therein, they exhibit excellent durability against wet heat and are capable of maintaining the stable state of engagement for a long period without producing deterioration of strength and degradation of the material due to hydrolysis, particularly change in the form of engagement part, and securing the stable state of the tape to which the engagement part is attached, even when repeatedly left under the high-temperature and high-humidity atmosphere. Further, when the sewing threads are also manufactured from a hydrolysis-resistant synthetic resin material, it is possible to provide a fastener product of synthetic resin which hardly incurs breakage of the sewing threads. In the case of a slide fastener, when the core cords are also manufactured from a hydrolysis-resistant synthetic resin material, the attached state of coupling elements becomes more stable. Accordingly, they can be advantageously used as fastener products to be attached to clothes such as working clothes to be used in a clean room of a pharmaceutical factory and those used in a hospital, medical service sites, nursing facilities, and the like which are repeatedly subjected to a sterilization treatment with high-temperature and high-pressure steam.

When all the component parts of the fastener products are manufactured from an essentially identical hydrolysis-resistant synthetic resin material, they are recyclable and contribute greatly to the conservation of the earth's environment and the effective utilization of resources. Further, since the raw materials for the component parts are unified, it is relatively easy to recover the discarded fastener products and the discarded plastic materials.

### BRIEF DESCRIPTION OF THE DRAWINGS

Other objects, features, and advantages of the invention will become apparent from the following description taken together with the drawings, in which:
Fig. 1 is a plan view illustrating one basic form of a slide fastener made of a hydrolysis-resistant synthetic resin according to the present invention;
Fig. 2 is a plan view illustrating another form of the slide fastener made of a hydrolysis-resistant synthetic resin according to the present invention;
Fig. 3 is a plan view illustrating still another form of the slide fastener made of a hydrolysis-resistant synthetic resin according to the present invention;
Fig. 4 is a partially cutaway plan view illustrating another form of the slide fastener made of a hydrolysis-resistant synthetic resin according to the present invention;
Fig. 5 is a fragmentary plan view of a coiled coupling element provided with a core cord;
Fig. 6 is a fragmentary cross-sectional view illustrating one state of fixing the coiled coupling element provided with a core cord shown in Fig. 5 to a fastener tape;
Fig. 7 is a fragmentary cross-sectional view illustrating another state of fixing the coiled coupling element provided with a core cord shown in Fig. 5 to a fastener tape;
Fig. 8 is a fragmentary plan view of a coiled coupling element devoid of a core cord;
Fig. 9 is a fragmentary cross-sectional view illustrating a state of fixing the coiled coupling element shown in Fig. 8 to a fastener tape;
Fig. 10 is a fragmentary plan view of a zigzag-like coupling element;
Fig. 11 is a fragmentary cross-sectional view illustrating a state of fixing the zigzag-like coupling element shown in Fig. 10 to a fastener tape;
Fig. 12 is a graph showing the results of measurement of the lateral tensile strength of a fastener stringer of slide fasteners produced in the working example and the comparative example to be described hereinafter measured after repeated autoclaving (126°C x 30 minutes);
Fig. 13 is a graph showing the results of measurement of the sliding resistance during the opening motion of slide fasteners produced in the working example and the comparative example to be described hereinafter measured after repeated autoclaving (126°C x 30 minutes); and
Fig. 14 is a graph showing the results of measurement of the sliding resistance during the closing motion of slide fasteners produced in the working example and the comparative example to be described hereinafter measured after repeated autoclaving (126°C x 30 minutes).

### DETAILED DESCRIPTION OF THE INVENTION

The present inventors, after pursuing a diligent study on the use of the fastener products of synthetic resin such as a slide fastener of synthetic resin, a separable fastener of synthetic resin under the high temperature and high humidity atmosphere, have found that the fastener products as mentioned above made of a hydrolysis-resistant synthetic resin, particularly a synthetic resin having a carbodiimide-based hydrolytic stabilizing agent incorporated therein exhibit excellent durability against wet heat, are capable of maintaining the stable state of engagement without producing such defects as deterioration of strength and discoloration even when repeatedly left under the high-temperature and high-humidity atmosphere, fulfill such characteristics as mechanical properties, resistance to wear and durability to withstand the friction due to the sliding motion which are expected of any fastener products for a long period, and are recyclable as well. The present invention has been perfected as a result.

To be specific, the fundamental technical idea of the present invention consists in manufacturing the component parts of fastener products with a synthetic resin material which exhibits excellent resistance to moist heat and to hydrolysis. It is provided, however, that there are times when the slider itself should be manufactured from other synthetic resin or a metal, depending on the function or construction which is expected from the slide fastener. In this case, the slider can be manufactured from the material which is so needed. In the case of the slide fastener using the slider of this description, it is relatively easy to recover the slider selectively from the discarded slide fastener and the discarded plastic materials emanating from the production line can be wholly reclaimed.

Since the fastener products of synthetic resin of the present invention exhibit excellent durability against wet heat, they are capable of maintaining the stable state of engagement for a long period without producing degradation of the material due to hydrolysis, particularly change in the form of engagement parts such as coupling elements, and securing the stable state of the tape to which the engagement parts such as coupling elements are attached, even when repeatedly subjected to washing and autoclaving.

When the individual component parts of the fastener product are manufactured from the same chemical type of synthetic resin material, it is possible to provide recyclable fastener products of synthetic resin. Further when the cloths of clothing on which the fastener products are fitted are manufactured from the same chemical type synthetic resins as those of the fastener products, it is made possible to recycle the whole clothing having the fastener products attached thereto.

The hydrolysis-resistant synthetic resin material used in the present invention means a synthetic resin having a hydrolytic stabilizing agent incorporated therein. As the synthetic resin, various synthetic resin materials such as polyester, polycarbonate, a polymer blend of polycarbonate/polyester, and nylon may be used. Since polyester is commonly used as the raw material for the hydrolysis-resistant cloths of clothing, polyester such as polyethylene terephthalate (PET) and polybutylene terephthalate (PBT) is more preferable in terms of recycle use and such characteristics as mechanical properties, durability to withstand the friction due to the sliding motion and resistance to wear which are expected of any fastener products.

As hydrolytic stabilizing agents, bis-carbodiimides represented by the formulas R-N=C=N-R and R-N=C=N-R' is used. In the above formulas, R and R' represent C₄-C₂₀ substituted or unsubstituted alkyl groups, substituted or unsubstituted aryl groups, wherein substitutions being halogen atom, nitro group, amino group, sulfonyl group, hydroxyl group, alkyl group, or alkoxy group, and wherein R and R' may or may not be the same. As concrete examples of such compounds, 2,2',6,6'-tetraisopropyldiphenyl carbodiimide; a bis-carbodiimide produced by Rhein-Chemie GmbH of Germany and marketed under the trademark designation of STABAXOL, and aromatic polycarbodiimides such as 2,4-diisocyanate-1,3,5-tris(1-methylethyl) copolymer with 2,6-diisopropyldiisocyanate and benzene-2,4-diisocyanato-1,3,5-tris(1-methylethyl) homopolymer may be cited. Properly, a hydrolytic stabilizing agent may be added to the synthetic resin material in an amount of about 1 to 5% by weight, preferably 1.5 to 2.5% by weight.

The hydrolytic stabilizing agent mentioned above is generally produced as a masterbatch made of a carrier resin and a hydrolytic stabilizing agent. For instance, the masterbatch may comprise about 70 to 98% by weight of a carrier resin and about 2 to 30% by weight of a hydrolytic stabilizing agent. The most preferable proportion is 15% by weight of the hydrolytic stabilizing agent to 85% by weight of the carrier resin. The carrier resin is preferred to be the same chemical type as a synthetic resin material.

Monofilaments or multifilaments may be produced by kneading such hydrolytic stabilizing agent-containing masterbatch chips and synthetic resin pellets and melt-extruding the resultant blend. They are used for weaving and/or knitting a fastener tape of a slide fastener and manufacturing sewing threads and core cords according to the present invention. Coiled coupling elements of a slide fastener may be manufactured from the monofilament. Further, coupling elements may be formed by injection molding.

Now, the modes of embodying the present invention in the component parts of the fastener products will be specifically described below with reference to various fastener products which are illustrated in the accompanying drawings.

Fig. 1 illustrates a slide fastener 1 which is used for opening and closing the opening in a garment or a bag and depicts the form of a product having the upper and lower ends of laterally paired fastener stringers 2 cut off. The fastener stringers 2 are composed of fastener tapes 3 made of hydrolysis-resistant synthetic resin and a row of coupling elements (coiled coupling elements) 4 made of hydrolysis-resistant synthetic resin attached fast to each of the opposed longitudinal edges of the fastener tapes 3. The fastener tapes 3 are formed by weaving and/or knitting hydrolysis-resistant synthetic resin fibers, manufactured from a non-woven fabric, or made of a sheet of hydrolysis-resistant synthetic resin. The coupling elements 4 are known in various forms such as, for example, those of the type obtained by injection molding the individual coupling elements and simultaneously attaching them fast to the edges of the fastener tapes, the continuous coupling elements such as the coiled coupling elements obtained by winding a monofilament of hydrolysis-resistant synthetic resin in the shape of a coil and the so-called zigzag coupling elements obtained by alternately connecting vertically in a zigzagging pattern in the longitudinal direction the portions bent in the shape of a letter U in the lateral direction in a plane, and the extrusion molded coupling elements obtained by attaching the opposite end portions of the individual coupling elements by means of extrusion molding to the two separate connecting cords (core cords) laid parallel to each other in the longitudinal direction thereby forming a composite resembling a ladder and bending the composite in the shape of a letter U around the longitudinal center line thereof. These examples of various coupling elements will be described afterward with reference to the relevant drawings. Then, the coiled coupling elements which include a core cord and a sewing thread among the component parts thereof will be also described afterward with reference to the relevant drawings. The reference numeral 5 denotes a slider which is slidable along the opposed rows of coupling elements for making and breaking engagement of the coupling elements.

A slide fastener 1a illustrated in Fig. 2 is in a form having the upper ends of the two fastener stringers 2 cut off. It is different from the slide fastener illustrated in Fig. 1 in respect that a lower stopping part 6 is formed by fusing the prescribed lower portions of the engaged rows of coupling elements 4.

A slide fastener 1b illustrated in Fig. 3 is different from the slide fastener illustrated in Fig. 1 in respect that upper stop members 7 are attached respectively to the upper ends of the rows of coupling elements 4b attached fast to fastener tapes 3b of fastener stringers 2b and a lower stop member 8 is attached to the lower ends thereof. The upper and lower stop members mentioned above are manufactured from a hydrolysis-resistant synthetic resin material.

Fig. 4 illustrates an open-link type slide fastener 1c. To the lower end portions of fastener tapes 3c of fastener stringers 2c, reinforcing sheet-like members (taffeta) 9 made of hydrolysis-resistant synthetic resin are welded through the medium of an adhesive layer (not shown). A box member 11 of a pin-and-box separator 10 made of hydrolysis-resistant synthetic resin is attached to the inner edge of one of the opposed reinforcing sheet-like members 9 and a butterfly rod or pin 17 made of hydrolysis-resistant synthetic resin is attached to the inner edge of the other reinforcing sheet-like member 9. The box member 11 is formed integrally with a guide projecting part 13 adjoining the box member 11 and a box rod 12 and a groove 14 is formed as interposed between the box rod 12 and the guide projecting part 13 so as to admit therein the lower end part of the slider 5 by slippage. Similarly, a guide groove 19 is formed between the butterfly rod 17 and a guide ridge 18 formed integrally with the adjoining butterfly rod 17. A butterfly rod inserting hole 15 is formed as pierced in the vertical direction in the left side portion of the box member 11 and a lateral groove 16 is formed on the outer wall of the butterfly rod inserting hole 15. When the butterfly rod 17 is inserted into the butterfly rod inserting hole 15 of the box member 11, therefore, the insertion can be smoothly carried out because the inner side of the lower end of the guide ridge 18 slide on the edge of the lateral groove 16 of the box member 11 so as to guide the butterfly rod 17.

With reference to Fig. 4, the reference numeral 20 denotes a core cord which is inserted in the longitudinal direction through the empty space inside the spiral of the coiled coupling element 4c and the reference numeral 21 denotes a sewing thread sewing the core cord 20 and the coiled coupling element 4c along the longitudinal edge of the fastener tape 3c. Both of them are manufactured from a hydrolysis-resistant synthetic resin material.

The pin-and-box separator does not need to be limited to what is illustrated in Fig. 4. The so-called reverse open-link type using the same box member as in the construction of the slider 5 and enabling the slider fastener to effect junction and disjunction of the opposed rows of coupling elements at the lower end thereof, for example, has been known as one version thereof.

Further, the embodiment, as illustrated in the diagram, uses reinforcing sheet-like members which are formed separately of the pin-and-box separator and welded to the lower end portion of each of the fastener tapes. The reinforcing sheet-like members do not need to be limited to this particular construction. The reinforcing members can be integrally formed with the pin-and-box separator as found, for example, in a construction which has a sheet-like portion produced by injection molding a synthetic resin material integrally with a box member or a butterfly rod and fixed to the entire width of the fastener tape or a construction which has slits of an arbitrarily selected pattern inserted in a sheet-like portion thereby imparting flexibility thereto.

Fig. 5 through Fig. 9 illustrate examples of coupling elements which are formed by coiling a monofilament of hydrolysis-resistant synthetic resin. Fig. 6 illustrates an example of having sewn to the longitudinal edge of a fastener tape 3d with a sewing thread 21 of hydrolysis-resistant synthetic resin a coiled coupling element 4d having the core cord 20 inserted through the empty space within a spiral in the longitudinal direction as illustrated in Fig. 5. In contrast, Fig. 7 illustrates an example of having a coiled coupling element 4e attached to the longitudinal edge of a fastener tape 3e as encircled with the tape at the same time that the tape is woven. Fig. 9 illustrates an example of having sewn to the longitudinal edge of a fastener tape 3f with the sewing thread 21 a coiled coupling element 4f having no core cord inserted through the empty space within a spiral as illustrated in Fig. 8.

Fig. 10 illustrates a so-called zigzag coupling element 4g which is obtained by forming U-shaped bends of a monofilament of hydrolysis-resistant synthetic resin each lying laterally in a plane and alternately connecting the U-shaped bends vertically in the longitudinal direction. The vertically adjacent bends are sewn with the sewing thread 21 to the longitudinal edge of a fastener tape 3g nipped therebetween.

The selection of the type of slide fastener product for proper application of the material depends also on the kind of synthetic resin to be used for the product. Generally, nylon 6 and nylon 66 among other polyamide resins are suitable for such slide fasteners as are shown in Fig. 1 through Fig. 16 and nylon 11 and nylon 12 are suitable for the railed fastener product. The polyester resins are suitable for both the slide fasteners and the railed fasteners.

When the synthetic resin material is polyethylene terephthalate (PET), basically the PET can be used for all the component parts of fastener products. In the case of a slide fastener, however, preferably the slider which is required to possess high mechanical strength is made of polybutylene terephthalate (PBT) instead, with the PBT in the body portion of the slider reinforced with such reinforcing fibers as glass fibers. In recycling the slide fastener of polyester answering this description, it is preferable to remove the slider from the slide fastener discarded as no longer useful and utilize the remainder of the slide fastener exclusively for the sake of reclamation. When the used slide fastener is wholly recovered and put to reclamation, the material that is obtained at all is in the form of a PET/PBT polymer blend. In the case of such an open-link type slide fastener as illustrated in Fig. 4, the pin-and-box separator is preferred to be made of PBT likewise on account of mechanical strength.

In any of the cases mentioned above, however, the component parts of the fastener products can be simultaneously dyed in the same hue by piece dyeing because the materials for the component parts are invariably polyester. Though various dyes are usable for the piece dyeing, a disperse dye is used preferably. The disperse dye that can be used herein is known in various types such as, for example, quinone type disperse dyes, azo type disperse dyes, and anthraquinone type disperse dyes. Various dyeing assistants in popular use such as leveling agents and dye fastness promotors can be additionally incorporated in a dye bath as is usually practiced. While various methods are available for the dyeing under discussion, the method of beam dyeing proves to be advantageous.

In setting the used polyester fastener products to the process of recycle, the reclaimed polyester may be used for manufacturing the fastener products such as slide fasteners again or for manufacturing other textile products and molded articles such as binding bands for packages and containers. When the reclaimed polyester is used as the raw material for other molded articles, it may incorporate therein a varying filler like such reinforcing fibers as glass fibers, carbon fibers, or aramid fibers or it may be blended with such other thermoplastic resin as PBT. In manufacturing a slide fastener by using reclaimed PET, the slider, pin-and-box separator, coupling elements, and sewing thread which require high mechanical strength are preferred to use virgin PET or a blend of virgin PET with reclaimed PET.

When the synthetic resin material is a polyamide, all the component parts of fastener products except a slider of a slide fastener, i.e. fastener tapes, coupling elements, a pin-and-box separator, reinforcing sheet-like members, upper and lower stop members, sewing threads, and core cords of a slide fastener can be made of the polyamide. The slider in a slide fastener can be made of the PBT mentioned above or a metal. When the slide fastener of polyamide answering this description is used in the recycling path, the slider is removed from the used slide fastener and the remainder of slide fastener is recycled. As concrete examples of the use found for the reclaimed polyamide, the component parts of a slide fastener excepting a slider, separable fasteners, snap tapes and other similar fastener products, textile products, and molded articles may be cited. In the case of the fastener products made of polyamide, similarly to the fastener products made of polyester mentioned above, the component parts made of polyamide can be simultaneously dyed in the same hue by piece dyeing. As concrete examples of the polyamide which is advantageously used herein, nylon 6, nylon 66, and copolymerized nylon may be cited.

When the cloths, such auxiliary materials as lining cloths, core cloths, and sewing threads, and such resinous accessories as buttons and snaps for garments on which the recyclable fastener product made of a synthetic resin according to the present invention is fitted are made of the same or homologous hydrolysis-resistant synthetic resin as that of the fastener product, it is made possible to recover the used products wholly and utilize them for reclamation without requiring the individual component parts thereof to be separated and selected.

The regeneration of the slide fastener from a discarded PET material is advantageously attained by granulating the recovered PET to strand-like chips, subjecting the chips to drying under a vacuum and, as occasion demands, to solid-phase polymerization, and extrusion molding the resultant polymer into a monofilament. Otherwise, the polymer may be molded into a sewing thread or multifilaments of a minute diameter. Alternatively, the polymer may be injection molded to form other component parts. In the case of a slide fastener, subsequently, the extrusion molded monofilament is drawn, formed in the shape of a coil, sewn to the edges of fastener tapes obtained by weaving and/or knitting PET fibers with the sewing thread, then heat set, and thereafter dyed to a desired color by piece dyeing. What is important in this operation is that the water content of the dry chips be repressed to the lowest possible extent and the decline of the intrinsic viscosity (I.V.) or limiting viscosity number before and after the work of monofilament extrusion be restrained for ensuring manufacture of fastener stringers of prescribed quality. The decline of the intrinsic viscosity before and after the work of monofilament extrusion is considered to originate in the hydrolysis of the resinous material caused by the water contained in the chips and is liable to induce breakage of the monofilament during the course of drawing. The water content of the dry chips, therefore, should be restrained 50 ppm (0.005%) and less, preferably 30 ppm and less, and more preferably 20 ppm and less. Particularly, in the manufacture of such products as sewing threads and multifilaments which have minute diameters, the water content should be kept 20 ppm and less, preferably 10 ppm and less, and more preferably 5 ppm and less in consideration of the possibility of breakage thereof.

Now, the present invention will be described specifically below with reference to working example.

### Example

Monofilaments manufactured from a mixture of PET and masterbatch chips (STABAXOL® KE9291 of Rhein-Chemie GmbH, consisting of a carrier resin PET (containing 5% of PE) containing 15% by weight of aromatic polycarbodiimide (STABAXOL® P100)) in a weight ratio of 7:1 were formed into coiled coupling elements. Fastener tapes were prepared by weaving PET high-tenacity yarn (BRABER® of Asahi Kasei Kogyo R.K., containing no hydrolytic stabilizing agent) and sewing threads and core cords were also manufactured from the same PET high-tenacity yarn. A slide fastener as shown in Fig. 1 was produced by using these component members.

### Comparative Example

A slide fastener was produced by following the procedure of Example except that only PET was used as a raw material for coiled elements.

### Test Example

Each of the slide fasteners prepared in Example and Comparative Example mentioned above was repeatedly subjected to autoclaving (126 °C x 30 minutes) and then tested for lateral tensile strength of a fastener stringer and for resistance to sliding motion when opening and closing a slide fastener in accordance with the methods described in JIS (Japanese Industrial Standard) S 3015. The measurement results of the lateral tensile strength are shown in Fig. 24, the measurement results of the resistance to sliding motion when opening the slide fastener in Fig. 25, and the measurement results of the resistance to sliding motion when closing the slide fastener in Fig. 26.

The guarantee value specified as the lateral tensile strength of a fastener stringer is 60 kg and over. Although the slide fasteners prepared in Example and Comparative Example satisfied this requirement even after 50 rounds of autoclaving, the slide fastener prepared in Comparative Example by using coiled elements manufactured from PET only had poor strength so as to cause breakages of coupling elements and sewing threads used for sewing coupling elements.

The guarantee value specified as the resistance to sliding motion in opening (when opening the slide fastener with a slider) and closing (when closing the slide fastener with a slider) is 700 g and under, respectively. Although the slide fastener prepared in Example satisfied this requirement even after about 100 rounds of autoclaving, the slide fastener prepared in Comparative Example had a value far from this guarantee value and its coupling elements had coarse surfaces containing a plenty of cracks with hangnails.

Further, when fastener tapes, sewing threads and core cords all manufactured from hydrolytic stabilizing agent-containing polyester fibers were used to prepare a slide fastener, the durability of the slide fastener against autoclaving has been further improved.

While certain specific embodiments and working example have been disclosed herein, the invention may be embodied in other specific forms. The described embodiments and example are therefore to be considered in all respects as illustrative and not restrictive, the scope of the invention being indicated by the appended claims rather than by the foregoing description.

## Claims

1. A slide fastener (1) made of a synthetic resin, comprising a pair of fastener tapes (3) and coupling elements (4) fixed to edges of said fastener tapes (3), wherein said fastener tapes (3) and said coupling elements (4) are made of a synthetic resin material containing a bis-carbodiimide as a hydrolytic stabilising agent and said coupling elements are continuous coupling elements in a coiled or zigzag form.

2. The slide fastener (1) according to claim 1, which further comprises sewing threads (21) for fixation of said coupling elements (4) to said fastener tapes (3), said sewing threads (21) being made of a synthetic resin material containing a bis-carbodiimide as a hydrolytic stabilising agent.

3. The slide fastener (1) according to claim 1 or 2, which further comprises core cords (20) extended as inserted through the individual coupling elements (4) in the longitudinal direction of said elements (4), said core cords (20) being made of a synthetic resin material containing a bis-carbodiimide as a hydrolytic stabilising agent.

4. The slide fastener (i) according to any one of claims 1 to 3, which further comprises upper and lower stop members (7,8) fitted respectively to upper and lower ends of said coupling elements (4), said upper and lower stop members (7,8) being made of a synthetic resin material containing a bis-carbodiimide as a hydrolytic stabilising agent.

5. The slide fastener (1) according to any one of claims 1 to 4, which is an open-link type slide fastener having a pin-and-box separator (10) and a pair of reinforcing sheet-like members (9) fixed respectively to lower end portions of said fastener tapes (3c), but having no lower stop member, wherein said pin-and-box separator (10) and reinforcing sheet-like members (9) being made of a synthetic resin material containing a bis-carbodiimide as a hydrolytic stabilising agent.

6. The slide fastener (1) according to claim 5, wherein said reinforcing sheet-like members (9) are integrated with said pin-and-box separator (10).

7. The slide fastener (i) according to any one of claims 1 to 6, wherein all component parts are made of the same chemical type of synthetic resin material.

8. The slide fastener (i) according to claim 7, wherein said synthetic resin material is polyester having a carbodiimide-based hydrolytic stabilizing agent incorporated therein.

9. The slide fastener (1) according to any one of claims 1 to 8, wherein said synthetic resin material contains 1 to 5% by weight of the bis-carbodiimide.

## Patentansprüche

1. Reißverschluss (1) aus einem Kunstharz, umfassend ein Paar Tragbänder (3) und an Kanten der Tragbänder (3) befestigte Kopplungselemente (4), wobei die Tragbänder (3) und die Kopplungselemente (4) aus einem Kunstharzmaterial gefertigt sind, das ein bis-Carbodiimid als ein hydrolytisches Stabilisierungsmittel enthält, und die Kopplungselemente fortlaufende Kopplungselemente in Spiral- oder Zickzackform sind.

2. Reißverschluss (1) nach Anspruch 1, welcher weiterhin Nähfäden (21) zur Befestigung der Kopplungselemente (4) an den Tr-agbändern (3) umfasst, wobei die Nähfäden (21) aus einem Kunstharzmaterial gefertigt sind, das ein bis-Carbodiimid als ein hydrolytisches Stabüisierungsmittel enthält.

3. Reißverschluss (1) nach Anspruch 1 oder 2, welcher weiterhin Kemkordein (20) umfasst, ausgedehnt wie eingeführt durch die einzelnen Kopplungselemente (4) in der Längsrichtung der Elemente (4), wobei die Kernkordeln (20) aus einem Kunstharzmaterial gefertigt sind, das ein bis-Carbodiimid als ein hydrolytisches Stabilisierungsmittel enthält.

4. Reißverschluss (1) nach einem der Ansprüche 1 bis 3, welcher weiterhin ein oberes und ein unteres Anschlagteil (7, 8) umfasst, die jeweils an das obere und das untere Ende der Kopplungselemente (4) angefügt sind, wobei das obere und das untere Anschlagteil (7, 8) aus einem Kunstharzmaterial gefertigt sind, das ein bis-Carbodiimid als ein hydrolytisches Stabilisierungsmittel enthält.

5. Reißverschluss (1) nach einem der Ansprüche 1 bis 4, welcher ein teilbarer Reißverschluss ist, der eine Steckteil-und-Kasten-Trenneinrichtung (10) und ein Paar flächenartiger Verstärkungsteile (9), die jeweils an unteren Endabschnitten der Tragbänder (3c) befestigt sind, aufweist, der aber kein unteres Anschlagteil besitzt, wobei die Steckteil-und-Kasten-Trenneinrichtung (10) und die flächenartigen Verstärkungsteile (9) aus einem Kunstharzmaterial gefertigt sind, das ein bis-Carbodiimid als ein hydrolykisches Stabilisierungsmittel enthält.

6. Reißverschluss (1) nach Anspruch 5, wobei die flächenartigen Verstärkungsteile (9) mit der Steckteil-und-Kasten-Trenneinrichtung (10) integriert sind.

7. Reißverschluss (1) nach einem der Ansprüche 1 bis 6, wobei alle Bestandteile aus Kunstharzmaterial des gleichen chemischen Typs gefertigt sind.

8. Reißverschluss (1) nach Anspruch 7, wobei das Kunstharzmaterial Polyester ist, in das ein auf Carbodiimid beruhendes hydrolytisches Stabilisierungsmittel eingegliedert ist.

9. Reißverschluss (1) nach einem der Ansprüche 1 bis 8, wobei das Kunstharzmaterial 1 bis 5 Gew.-% des bis-Carbodiimids enthält.

## Revendications

1. Fermeture à glissière (1) en résine synthétique, comprenant une paire de rubans de fermeture (3) et des éléments d'accouplement (4) fixés aux bords desdits rubans de fermeture (3), lesdits rubans de fermeture (3) et lesdits éléments d'accouplement (4) étant faits d'un matériau de type résine synthétique contenant un bis-carbodiimide en tant qu'agent de stabilisation vis-à-vis de l'hydrolyse, et lesdits éléments d'accouplement étant des éléments d'accouplement continus sous forme de spirale ou en zigzag.

2. Fermeture à glissière (1) selon la revendication 1, comprenant en outre des fils de couture (21) qui fixent lesdits éléments d'accouplement (4) sur les rubans de fermeture (3), lesdits fils de couture (21) étant faits d'un matériau de type résine synthétique contenant un bis-carbodiimide en tant qu'agent de stabilisation vis-à-vis de l'hydrolyse.

3. Fermeture à glissière (1) selon la revendication 1 ou 2, comprenant en outre des cordons centraux (20) insérés dans les éléments d'accouplement individuels (4) dans la direction longitudinale desdits éléments (4), lesdits cordons centraux (20) étant faits d'un matériau de type résine synthétique contenant un bis-carbodiimide en tant qu'agent de stabilisation vis-à-vis de l'hydrolyse.

4. Fermeture à glissière (1) selon l'une quelconque des revendications 1 à 3, comprenant en outre des éléments d'arrêt supérieurs et inférieur (7, 8) montés respectivement sur les extrémités supérieure et inférieure desdits éléments d'accouplement (4), lesdits éléments d'arrêt supérieurs et inférieur (7, 8) étant faits d'un matériau de type résine synthétique contenant un bis-carbodiimide en tant qu'agent de stabilisation vis-à-vis de l'hydrolyse.

5. Fermeture à glissière (1) selon l'une quelconque des revendications 1 à 4, qui est une fermeture à glissière du type à lien ouvert comportant une butée séparable (10) et une paire d'éléments de renforcement de type ruban (9) fixés respectivement aux parties d'extrémité inférieure desdits rubans de fermeture (3c), mais n'ayant pas d'élément d'arrêt inférieur, ladite butée séparable (10) et lesdits éléments de renforcement de type ruban (9) étant faits d'un matériau de type résine synthétique contenant un bis-carbodiimide en tant qu'agent de stabilisation vis-à-vis de l'hydrolyse.

6. Fermeture à glissière (1) selon la revendication 5, dans laquelle lesdits éléments de renforcement de type ruban (9) sont intégrés à ladite butée séparable (10).

7. Fermeture à glissière (1) selon l'une quelconque des revendications 1 à 6, dans laquelle toutes les parties constitutives sont faites du même type chimique de matériau de type résine synthétique.

8. Fermeture à glissière (1) selon la revendication 7, dans laquelle ledit matériau de type résine synthétique est du polyester dans lequel est incorporé un agent de stabilisation vis-à-vis de l'hydrolyse à base de carbodiimide.

9. Fermeture à glissière (1) selon l'une quelconque des revendications 1 à 8, dans laquelle ledit matériau de type résine synthétique contient de 1 à 5 % en poids de bis-carbodiimide.
